

Dec. 29, 1970

R. G. BARKER

3,551,286

POLYSULFIDE PAPER PULPING COMPOSITION

Filed Jan. 3, 1968

COMPARISON OF TOTAL YIELD FOR  
COMPOSITION OF THIS INVENTION  
AND FOR PRIOR ART



INVENTOR  
RICHARD G. BARKER

BY

Kane, Palmer, Kane, Sullivan & Smith  
ATTORNEYS

## 1

3,551,286

**POLYSULFIDE PAPER PULPING COMPOSITION**  
Richard G. Barker, Princeton Junction, N.J., assignor to  
Union Camp Corporation, New York, N.Y., a corporation  
of Virginia  
Continuation-in-part of application Ser. No. 620,288,  
Mar. 3, 1967. This application Jan. 3, 1968, Ser.  
No. 695,495  
The portion of the term of the patent subsequent to  
Sept. 30, 1986, has been disclaimed  
Int. Cl. D21c 3/00

U.S. CL. 162—82

6 Claims

**ABSTRACT OF THE DISCLOSURE**

An aqueous, alkaline modified kraft pulping solution for obtaining increased cellulose yield in paper pulping, while minimizing corrosion and air pollution, comprising a total sulfur content of from 5 to 60 grams per liter, said sulfur consisting of from 43 to 80 percent from an alkali metal polysulfide, from 40 to 15 percent from an alkali metal sulfide, and up to 17 percent from an alkali metal thiosulfate, particularly a pulping solution, the active inorganic constituents of which are recirculated for additional pulping, after recovery.

**CROSS-REFERENCES TO RELATED APPLICATIONS**

This application is a continuation-in-part of my copending application, Ser. No. 620,288, filed Mar. 3, 1967, for "Sodium Polysulfide Pulping Process and Regeneration," now Pat. No. 3,470,061.

**BACKGROUND OF THE INVENTION**

The kraft process is the most extensively employed for the pulping of lignocellulosic materials. The active ingredients used for digestion in the kraft process are sodium hydroxide and sodium sulfide in a strongly alkaline, aqueous solution. Almost any wood species, for example, slash pine, can be pulped by this process.

The total sulfur content of the kraft pulping, or white, liquor, is generally between about 5 and 60 grams per liter. Most often, and preferably, it is in the range of from 10 to 30 grams per liter. This white liquor is usually diluted with water, or spent pulping liquor, before addition to a charge of wood chips and the mixture of wood chips and pulping liquor is then heated, under pressure, at a temperature of 150° C. to 190° C. for digestion.

The kraft pulps show wide variations in the lignin content, and the cellulose yield is different for each such lignin content. It is obviously desirable to increase the pulp yield, for any given lignin content, as this means that an increased amount of pulp is derived from a given wood charge. Polysulfide pulping has previously been disclosed as a way to improve this yield. Inclusion of polysulfide sulfur in the kraft white liquor increases the carbohydrate retention of the wood charge, and thereby increases the pulp yield. This has been previously demonstrated, for example, in U.S. Pat. No. 3,216,887—Landmark and U.S. Pat. No. 2,944,928—Kibrick et al.

However, an increase in the polysulfide content of the white liquor, though improving the yield, has meant an increase in the total sulfur content of the white liquor. Further, in pulping, the polysulfide is converted to sulfide so that the spent liquor has a higher concentration of sulfide than would otherwise be true. If the inorganic constituents of the liquor are then recirculated, after recovery, for additional pulping, and the polysulfide concentration is again increased, the total sulfur content is increased still further, leading to severe problems.

## 2

As is well known, increased sulfur content increases corrosion of pulp processing equipment and, perhaps more importantly, greatly increases the sulfur losses to the atmosphere, contributing drastically to air pollution.

The solution to the problem, and an object of this invention is to provide a pulping solution, particularly one where the inorganic constituents can be recovered and recirculated, where the polysulfide content is increased so as to increase the pulp yield, while maintaining a total sulfur concentration within acceptable limits as to corrosion and pollution. Such a composition is not described in either of the two previously mentioned prior art patents, nor can such a composition be attained by following the disclosures in those patents.

**SUMMARY OF THE INVENTION**

In accordance with the present invention, an aqueous pulping solution is employed having between 5 and 60 grams per liter of sulfur, more preferably between 10 and 30 grams per liter. While the higher total sulfur range can be employed within the present invention, limiting the maximum sulfur content to 30 grams per liter avoids excessive corrosion and pollution problems. The desired pulping action is not obtained with sulfur concentrations below about 5 grams per liter.

As important as the total sulfur content, is the source of this sulfur. According to the present invention, from 43 to 80 percent of the total sulfur content is obtained from an alkali metal polysulfide, preferably sodium polysulfide. The sodium polysulfide is preferred because of its significantly lower cost and easier recovery. More preferably, from 50 to 70 percent of the total sulfur content is derived from the alkali metal polysulfide.

Between about 40 and 15 percent of the total sulfur should be derived from an alkali metal sulfide. As sodium polysulfide is the preferred alkali metal polysulfide, the preferred sulfide is sodium sulfide. More preferably, the percentage of sulfur obtained from the alkali metal sulfide is between about 40 and 17 percent.

The third major sulfur-containing constituent of the system is an alkali metal thiosulfate, generally sodium thiosulfate because of the constituency of the other two sulfur-containing materials. While the alkali metal thiosulfate has no real function in the pulping process, it results from the use of the other materials and is, preferably, maintained at as low a level as possible. According to the present invention, this level is generally less than about 17 percent, and preferably less than about 10 percent.

The pulping solution must also contain a certain amount of alkali. The amount of alkali contained in the pulping solution is not critical and the solution is effective for pulping with, for example, a total alkali content of from 15 to 400 grams per liter, as Na<sub>2</sub>O. More preferably, the total alkali content is from 70 to 120 grams per liter. This alkali is generally derived from the group consisting of sodium hydroxide, sodium carbonate, and sodium sulfide.

**BRIEF DESCRIPTION OF THE DRAWINGS**

The figure is a plot of yield compared to Kappa number showing the improved yields obtained with a composition of the present invention as opposed to those of a prior art composition.

**DESCRIPTION OF THE PREFERRED EMBODIMENTS**

In my aforementioned copending application, Ser. No. 620,288, filed Mar. 3, 1967, I have described a process for oxidizing a white liquor or white liquor-black liquor

mixture in order to convert the alkali metal sulfide, particularly sodium sulfide, to an alkali metal polysulfide, particularly sodium polysulfide. According to that application, various solid, inorganic manganese oxidizers can be employed, including  $Mn_2O_3$ ,  $Mn_3O_4$ ,  $MnS_2$ , partially oxidized  $MnO$ ,  $MnOOH$ , and  $MnO_2$ , and the oxidation takes place at a temperature in the range of from 40° to 120° C. The pulping compositions of the present invention can be maintained, recirculating the active inorganic constituents of the pulping solution, by employing the process of that aforementioned application. By that process, the polysulfide level can be brought within the desired range without increasing the alkali metal thiosulfate level beyond that desired and without the addition of alkali metal polysulfide. Thus, the total sulfur content is not raised beyond the desired level, ameliorating the corrosion and pollution problems.

Employing the pulping composition of the present invention, significantly improved yields are obtained. This is true with respect to the standard kraft composition, as well as by comparison with the prior art processes.

These improvements will be described in greater detail in the following examples. These examples should be considered as illustrative only, and not as limiting in any way the full scope of the invention as covered in the appended claims.

#### EXAMPLE 1

In this example the pulping composition of the present invention was employed, and compared with a standard kraft pulping composition, on slash pine to obtain a pulp with a Kappa value of about 100. The compositions of the two pulping solutions, with respect to total sulfur content, are shown below, both as grams per liter of sulfur obtained from the particular component, and as to the sulfur percentage obtained from each sulfur-bearing component.

TABLE I

| Sulfur-bearing component | Sulfur in kraft pulping composition |                         | Sulfur in pulping composition of the present invention |                         |
|--------------------------|-------------------------------------|-------------------------|--------------------------------------------------------|-------------------------|
|                          | Grams per liter                     | Percent of total sulfur | Grams per liter                                        | Percent of total sulfur |
| Sodium polysulfide.....  | 0                                   | 0                       | 7.52                                                   | 46                      |
| Sodium sulfide.....      | 16.4                                | 100                     | 6.08                                                   | 37                      |
| Sodium thiosulfate.....  | 0                                   | 0                       | 2.8                                                    | 17                      |

Employing these two compositions to pulp slash pine obtained from the same batch, with an active alkali content in the pulping solution, in each case, of about 100 grams per liter, expressed as  $Na_2O$ , and using a digesting temperature of 160° C., the yield with the composition of the present invention was approximately 2 percent greater, and with a lower Kappa value. Specifically, the standard kraft composition gave a 56.8 percent yield with a Kappa number of 111, while the process employing the composition of the present invention resulted in a 58.5 percent yield, with a Kappa number of 101. The sodium sulfide concentration in the black liquor was 7.8 grams per liter for the kraft process and 8.1 grams per liter for the process employing the composition of the present invention. Thus, the yield improvement obtained with the composition of the present invention was gained without a significant increase in the final sulfur content, and the attendant problems of increased corrosion and pollution.

#### EXAMPLE 2

A comparison, similar to that in Example 1, was made between the composition of the present invention and a kraft pulping composition in producing a pulp with a Kappa number of approximately 130. The pulping com-

positions as shown in the table below, in the same manner as in Table I of Example 1:

TABLE II

| Sulfur-bearing component | Sulfur in kraft pulping composition |                         | Sulfur in pulping composition of the present invention |                         |
|--------------------------|-------------------------------------|-------------------------|--------------------------------------------------------|-------------------------|
|                          | Grams per liter                     | Percent of total sulfur | Grams per liter                                        | Percent of total sulfur |
| Sodium polysulfide.....  | 0                                   | 0                       | 8.55                                                   | 52.1                    |
| Sodium sulfide.....      | 16.4                                | 100                     | 6.26                                                   | 38.2                    |
| Sodium thiosulfate.....  | 0                                   | 0                       | 1.59                                                   | 9.7                     |

A yield improvement of about 4 percent was realized in this example, the kraft composition providing a 60.3 percent yield of pulp with a Kappa number of 125, while the composition of the present invention showed a 64.6 percent pulp yield at a Kappa number of 135. Again, the pulping processes were carried out under similar conditions, each of the compositions having about 100 grams per liter of active alkali, expressed as  $Na_2O$ , with a digesting temperature of 160° C.

The kraft composition black liquor showed 6.5 grams per liter of sodium sulfide, while employing the composition of the present invention, a black liquor was obtained having a 4.8 grams per liter of sodium sulfide.

Thus, at both Kappa levels, when the composition of the present invention is compared with a standard kraft pulping composition, yields are improved without a correlated rise in the black liquor sodium sulfide concentration, so that corrosion and pollution problems are not increased along with the yield increase.

By comparison, the employment of the polysulfide composition of the prior art which, as previously mentioned, provided yield increases, also resulted in significant increases in the sodium sulfide level of the black liquid, representative of increased pollution and corrosion. This is illustrated in Example 3.

#### EXAMPLE 3

In this example a standard kraft composition was compared with a modified kraft composition where the kraft liquor contained sufficient polysulfide for an application of 1 percent polysulfide sulfur on the wood. These compositions are shown in Table III in the same manner as were the kraft composition and composition of the present invention in Table I of Example 1.

TABLE III

| Composition for 1 percent application of polysulfide sulfur | Sulfur in kraft pulping composition |                         | Sulfur in modified kraft composition |                         |
|-------------------------------------------------------------|-------------------------------------|-------------------------|--------------------------------------|-------------------------|
|                                                             | Grams per liter                     | Percent of total sulfur | Grams per liter                      | Percent of total sulfur |
| Sodium polysulfide.....                                     | 0                                   | 0                       | 8.8                                  | 37.3                    |
| Sodium sulfide.....                                         | 14.8                                | 100                     | 14.8                                 | 62.7                    |

Employing essentially the same conditions with the two pulping compositions at a digesting temperature of 173° C., the straight kraft composition yielded 57.8 percent pulp with a Kappa number of 99.3, while the modified composition yielded 59.0 percent pulp with a Kappa number of 97.5. Thus, there was a yield increase of a little over 1 percent. However, the sodium sulfide content of the black liquor was increased significantly, in fact, almost by a factor of 2. The content of sodium sulfide in the black liquor from the straight kraft composition was 6.6 grams per liter, while from the modified process it was 11.2 grams per liter. Employing this modified composition, not only would there be significantly increased corrosion, and significantly increased air pollution, but the cost of the process would additionally be raised due to the requirements for additional sulfur, including the losses resulting from such a high sulfur content in the black liquor.

5  
EXAMPLE 4

In this example, the composition of the present invention was compared with that of Landmark, where as significant percentage of the pulping composition sulfur is obtained from sodium polysulfide, but where that percentage is significantly lower than the percentages called for in the present invention. Similarly, in the Landmark composition the thiosulfate percentages are significantly higher. A composition was prepared according to the Landmark patent disclosure having 37 grams per liter of sodium sulfide, 30 grams per liter of sodium thiosulfate, and 7.28 grams per liter of polysulfide sulfur. The composition had an effective alkali content of 74 grams per liter, 88.7 grams per liter of active alkali. A composition was also prepared having 74 grams per liter of effective alkali and 33.8 grams per liter of sulfur, all obtained from sodium sulfide. This latter composition was then oxidized, employing the process of my aforementioned copending application, particularly using manganese dioxide at a temperature of 60° C. The resulting compositions, which were used for pulping, are as follows, with designations the same as those of Table I in Example 1:

TABLE IV

| Sulfur-bearing component | Sulfur in<br>landmark Pat.<br>No. 3,216,887<br>composition |                            | Sulfur in<br>pulping composi-<br>tion of the present<br>invention |                               |
|--------------------------|------------------------------------------------------------|----------------------------|-------------------------------------------------------------------|-------------------------------|
|                          | Grams<br>per<br>liter                                      | Percent<br>total<br>sulfur | Grams<br>per<br>liter                                             | Percent<br>of total<br>sulfur |
| Sodium polysulfide.....  | 7.28                                                       | 21.0                       | 25.12                                                             | 74.                           |
| Sodium sulfide.....      | 15.2                                                       | 43.9                       | 5.88                                                              | 17.4                          |
| Sodium thiosulfate.....  | 12.15                                                      | 35.1                       | 2.8                                                               | 8.3                           |
| Total sulfur.....        | 34.63                                                      | -----                      | 33.8                                                              | -----                         |

The above-mentioned compositions were employed to pulp slash pine chips, taken from the same batch, employing an impregnation time of 45 minutes and temperature of 110° C., and the same maximum pulping temperature of 160° C.

As can be seen from the figure, at equivalent Kappa numbers, the yields were significantly increased employing the composition of the present invention, as opposed to the composition of the Landmark patent. For example, at Kappa numbers between 40 and 45, the composition of the present invention gave pulp yields of between 55 and 56 percent, while the Landmark composition showed pulp yields between 53½ and 54½ percent.

Thus, employing the composition of the present invention, with the same total sulfur content as in a prior art composition with different constituent percentages, significantly increased yields are obtained. These increased yields are gained without an increase in corrosion and pollution problems, as the sulfur contents of the resulting black liquors are essentially the same.

The active inorganic constituents in the black liquor resulting from the composition of the present invention in this example can be recovered in normal fashion and the polysulfide content regenerated by treatment with

## 6

the manganese oxidant described in my aforementioned copending application. These inorganic constituents can then be recirculated for additional pulping. Thus, the pulping liquor composition can be maintained at approximately the levels shown in the table, adding only sufficient materials to make up for that lost through normal processing. As with standard pulping solutions, the composition of the present invention can also contain sodium carbonate and sodium sulfate, without interfering with normal processing.

The invention has been described in detail with particular reference made to various preferred embodiments thereof, but it will be understood that variations and modifications can be effected within the spirit and scope of the invention as described hereinabove and as defined in the appended claims.

I claim:

1. A sulfur-containing aqueous alkaline modified kraft pulping solution for the digestion of lignocellulosic materials for paper-making having a total sulfur content of from 5 to 60 grams per liter, said sulfur consisting of
  - (a) from 43 to 80 percent from an alkali metal polysulfide
  - (b) from about 15 to 40 percent from an alkali metal sulfide, and
  - (c) less than about 17 percent from an alkali metal thiosulfate.
2. The liquor of claim 1 containing from 15 to 400 grams per liter of total alkali, as N<sub>2</sub>O, said total alkali being derived from sodium hydroxide, sodium sulfide, and sodium carbonate.
3. The liquor of claim 2 having from 70 to 120 grams per liter of total alkali.
4. The liquor of claim 1 wherein said alkali metal is sodium and said total sulfur content is from 10 to 30 grams per liter.
5. The liquor of claim 4 wherein said sulfur consists of from about 50 to 75 percent as sodium polysulfide, from about 17 to 40 percent as sodium sulfide, and less than about 10 percent as sodium thiosulfate.
6. The liquor of claim 1 having from 70 to 120 grams per liter of total alkali, wherein said alkali metal is sodium and said total sulfur content is from 10 to 30 grams per liter and wherein said sulfur consists of from about 50 to 75 percent as sodium polysulfide, from about 17 to 40 percent as sodium sulfide, and less than about 10 percent as sodium thiosulfate.

## References Cited

## UNITED STATES PATENTS

- 3,216,887 5/1964 Lanomarr ----- 162-38  
3,470,061 9/1969 Barbor ----- 162-38

S. LEON BASHORE, Primary Examiner

R. H. ANDERSON, Assistant Examiner

U.S. Cl. X.R.

**Disclaimer**

3,551,286.—*Richard G. Barker*, Princeton Junction, N.J. POLYSULFIDE PAPER PULPING COMPOSITION. Patent dated Dec. 29, 1970. Disclaimer filed Aug. 1, 1973, by the assignee, *Union Camp Corporation*.

Hereby enters this disclaimer to claims 1 through 6, inclusive, of said patent. [Official Gazette December 25, 1973.]